# EUROPEAN PATENT SPECIFICATION

(11) **EP 1 602 784 B1**
(45) Date of publication and mention of the grant of the patent: **13.10.2010**
(21) Application number: 05252241.4
(22) Date of filing: 09.04.2005
(51) Int. Cl.: D21H 27/26, D21H 21/54, C08J 9/28

(54) **Method of preparing decorative laminate**
Verfahren zur Herstellung eines Dekorlaminats
Procédé de fabrication d'un stratifié décoratif

(30) Priority: 23.04.2004 EP 04291068
(43) Date of publication of application: 07.12.2005
(73) Proprietor: ROHM AND HAAS COMPANY, Philadelphia, Pennsylvania 19106-2399 (US)
(72) Inventor: Brown, James T., Bechtelsville, Pennsylvania 19505 (US); Haigh, John Robert, 6300 Roquefort Les Pins (FR)
(74) Representative: Buckley, Guy Julian

(56) References cited:
- US-A- 4 594 363
- US-A- 4 726 986
- US-A- 6 139 961

## Description

The present invention relates to a method of preparing a decorative laminate, using a hollow sphere polymer. In particular, the present invention relates to a method of preparing a decorative laminate, using a hollow sphere polymer whose void has been created by swelling the polymer with a fixed or permanent base; and further relates to a decorative laminate prepared by the method.

Voided, or hollow emulsion polymers are generally prepared by swelling a multi-stage polymer, having a core and a shell, in such a way that one or more voids form in the interior of the emulsion polymer particle. Hollow emulsion polymers are often used in paints, coatings, inks, sunscreens, paper manufacture, and several other industrial arenas. In the paper industry, hollow emulsion polymers are used to make the surface of the paper, among other things, smoother, brighter, and more opaque. Additional benefits of hollow sphere polymers is that, when used alone, or in combination with costly opacifying pigments, such as titanium dioxide, a more cost effective system is obtainable. The paper typically utilized during the manufacture of decorative laminates has a high pigment content. The pigment typically utilized is titanium dioxide, which, as mentioned above, is extremely costly. However, hollow emulsion polymers are not currently utilized to replace or complement such costly pigments during processing of the decorative laminate paper. This is due, in part, to the belief that the subjection of the opaque emulsion polymer to the conditions of processing of both the paper, and the decorative laminate, would eliminate the advantages normally associated with the use of opaque emulsion polymers.

U.S. Patent No. 4,594,363 discloses a process for making core/sheath polymer particles containing voids, including the step of swelling, at elevated temperature, the resultant core/sheath polymer particles with fixed or permanent base so as to produce a dispersion of particles which, when dried, contain a microvoid. However, the patent does not disclose a method of using the core/sheath polymer particles to make a decorative laminate.

U.S. Patent No. 6,139,961 discloses a method for improving the strength and opacity of paper or paperboard by applying to the paper, during wet-end processing of the paper, a hollow sphere organic polymer having a core, a hard polymer shell surrounding the core, and a soft polymer shell surrounding the first shell, wherein (1) the second shell polymer is at least 15% by weight of the total weight of the first shell polymer and the second shell polymer, (2) the second shell polymer has a glass transition temperature of less than 15°C, and (3) the polymer has been swollen by a volatile, or fixed or permanent base. However, the patent does not disclose use of a hollow sphere polymer to make a decorative laminate.

US 4 726 986 A1 discloses a resin impregnated and resin coated laminate comprising a core and a top decorative layer containing a decorative sheet having a top exterior coating thereon comprising hollow microspheres.

Applicants have unexpectedly discovered that hollow sphere polymers that have been swollen by a fixed or permanent base are useful for preparing decorative laminates, despite the subjection of the hollow sphere polymer to the harsh conditions, such as high temperatures and/or pressures, typically present during processing of a decorative laminate.

A first aspect of the present invention is a method of preparing a decorative laminate, comprising the steps of: (I) preparing a paper by (a) providing a hollow sphere polymer made by: (i) forming a core stage polymer by polymerizing at least one monoethylenically unsaturated monomer containing acid functionality, (ii) encapsulating said core stage polymer with at least one shell stage polymer, by emulsion polymerizing at least one shell stage monomer system in the presence of said core stage polymer, wherein said shell stage polymer permits penetration of a fixed or permanent base; (iii) contacting the resulting multi-stage polymer particles with fixed or permanent base, wherein either (1) said shell stage polymer comprises at least 1% acid functional monomer, or (2) said contacting takes place in the presence of solvent; (b) contacting said paper with a composition comprising said hollow sphere polymer and at least one pigment; and (c) drying said paper; (II) impregnating said paper with a crosslinking resin; (III) applying pressure to said paper; and (IV) exposing said paper to temperatures of from 100°C to 300°C.

A second aspect of the present invention is a decorative laminate formed by the method of the first aspect.

The method of the present invention is directed toward the preparation of a decorative laminate that contains a paper that has incorporated within it, a fixed or permanent base-swollen hollow sphere polymer. By "decorative laminate" is meant herein an article containing a decorative paper, which may or may not be printed or embossed, and that has within and/or upon it a hardened crosslinked resin. The first step of the method is the provision of a hollow sphere polymer that has been made by forming a multi-stage polymer having a core stage that is encapsulated by a shell stage, and then swelling the multi-stage polymer by contacting it with a fixed or permanent base, to form the hollow sphere polymer. Hollow sphere polymers of this type are well known in the art, and commercially available.

The core stage polymer is an emulsion polymer that has been formed by polymerizing at least one monoethylenically unsaturated monomer containing acid functionality. The core stage polymer is prepared by emulsion homo-polymerization of the acid-containing monomer, or by co-polymerization of the acid-containing monomer with at least one other acid-containing monomer. Suitable monoethylenicially unsaturated monomers containing acid functionality, useful for making the core stage polymer, include, for example, monomers containing at least one carboxylic acid group including acrylic acid, methacrylic acid, acryloxypropionic acid, (meth)acryloxypropionic acid, itaconic acid, aconitic acid, maleic acid or anhydride, fumaric acid, crotonic acid, monomethyl maleate, monomethyl fumarate, and monomethyl itaconate; also contemplated is the use of terminally unsaturated acid-containing oligomers such as, for example, are taught in US patents No. 5,710,227 and 6,046,278 and EP 1010706, and including comb/graft, block, and mixed block oligomers. The use of the term "(meth)" followed by another term such as acrylate, acrylonitrile, or acrylamide, as used throughout the disclosure, refers to both acrylate, acrylonitrile, or acrylamide and methacrylate, methacrylonitrile, and methacrylamide, respectively. Acrylic acid and methacrylic acid are preferred.

In general, core copolymers containing at least 5%, preferably at least 10%, by weight of the acid mers have practical swellability for the purposes of the present invention. However, there may be instances where, because of the hydrophobicity of certain comonomers, the copolymer may require more, or less, than 5 weight percent of acid-containing monomer. As noted above, the core stage polymer may be formed by homo-polymerization of an acid-containing monomer. Thus, the invention includes a core containing 100% of the emulsion polymerized acid-containing monomer. A preferred maximum quantity of acid-containing monomer is about 70%, by weight, of the total core stage monomers.

In a preferred embodiment, the acid-containing monomer is copolymerized with one or more nonionic monoethylenically unsaturated monomers. In one embodiment, the core stage polymer is formed by copolymerizing from 5 to 100%, preferably from 20% to 60%, and more preferably, from 30% to 50%, by weight, based on the weight of the core stage polymer, of at least one ethylenicially unsaturated monomer containing acid functionality, and from 0 to 95% by weight, based on the weight of the core stage polymer, of at least one nonionic monoethylenically unsaturated monomer. Suitable nonionic monoethylenically unsaturated monomers for making the core stage polymer include styrene, α-methyl styrene, p-methyl styrene, t-butyl styrene, vinyltoluene, ethylene, vinyl acetate, vinyl chloride, vinylidene chloride, (meth)acrylonitrile, (meth)acrylamide, (C₁-C₂₀) alkyl or (C₃-C₂₀) alkenyl esters of (meth)acrylic acid, such as methyl (meth)acrylate, ethyl (meth)acrylate, butyl (meth)acrylate, 2-ethylhexyl (meth)acrylate, hydroxyethyl(meth)acrylate, hydroxypropyl(meth)acrylate, benzyl (meth)acrylate, lauryl (meth)acrylate, oleyl (meth)acrylate, palmityl (meth)acrylate, stearyl (meth)acrylate and the like.

The core stage polymer may optionally contain less than 20% by weight, preferably from 0.1 to 3% by weight, based on the total weight of the core, of polyethylenically unsaturated monomer, wherein the amount used is generally approximately directly proportional to the amount of monoethylenically unsaturated acid-containing monomer used; in other words, as the relative amount of monoethylenically unsaturated acid-containing monomer increases, it is acceptable to increase the level of polyethylenically unsaturated monomer. Alternatively, the core polymer may contain from 0.1 to 60 % by weight, based on the total weight of the core polymer, of butadiene.

Suitable polyethylenically unsaturated monomers include comonomers containing at least two addition polymerizable vinylidene groups and are alpha beta ethylenically unsaturated monocarboxylic acid esters of polyhydric alcohols containing 2-6 ester groups. Such comonomers include alkylene glycol diacrylates and dimethacrylates, such as for example, ethylene glycol diacrylate, ethylene glycol dimethacrylate, 1,3-butylene glycol diacrylate, 1,4-butylene glycol diacrylate propylene glycol diacrylate and triethylene glycol dimethylacrylate; 1,3-glycerol dimethacrylate; 1,1,1-trimethylol propane dimethacrylate; 1,1,1-trimethylol ethane diacrylate; pentaerythritol trimethacrylate; 1,2,6-hexane triacrylate; sorbitol pentamethacrylate; methylene bis-acrylamide, methylene bis-methacrylamide, divinyl benzene, vinyl methacrylate, vinyl crotonate, vinyl acrylate, vinyl acetylene, trivinyl benzene, triallyl cyanurate, divinyl acetylene, divinyl ethane, divinyl sulfide, divinyl ether, divinyl sulfone, diallyl cyanamide, ethylene glycol divinyl ether, diallyl phthalate, divinyl dimethyl silane, glycerol trivinyl ether, divinyl adipate; dicyclopentenyl (meth)acrylates; dicyclopentenyloxy (meth)acrylates; unsaturated esters of glycol monodicyclopentenyl ethers; allyl esters of mono- and dicarboxylic acids having terminal ethylenic unsaturation including allyl (meth)acrylate, diallyl maleate, diallyl fumarate, diallyl itaconate and the like.

The shell stage of the hollow sphere polymer of this invention preferably has a relatively moderate to high glass transition temperature (Tg). Preferably, the outermost shell stage polymer Tg is greater then 25°C, more preferably greater than 50°C, even more preferably greater than 70°C, and most preferably greater than 90°C, as calculated by the Fox Equation (T.G. Fox, Bull. Am. Physics Soc., Volume 1, Issue No. 3, page 123 (1956)). That is, for calculating the Tg of a copolymer of monomers M1 and M2,$1 / Tg \left(calc.\right) = w \left(M⁢1\right) / Tg \left(M⁢1\right) + w \left(M⁢2\right) / Tg \left(M⁢2\right)$ wherein
Tg(calc.) is the glass transition temperature calculated for the copolymer
w(M1) is the weight fraction of monomer M1 in the copolymer
w(M2) is the weight fraction of monomer M2 in the copolymer
Tg(M1) is the glass transition temperature of the homopolymer of M1
Tg(M2) is the glass transition temperature of the homopolymer of M2,
all temperatures being in °K.

The shell stage polymer is the product of emulsion polymerizing a shell stage monomer system in the presence of the core stage polymer. The monomers used, and the relative proportions thereof in the shell stage polymer, should be such that the shell stage polymer permits permeation of a fixed or permanent base. It is preferred that the shell stage monomer system be all acrylic. However, in a particularly preferred embodiment, the shell stage polymer contains as copolymerized units butyl methacrylate, methyl methacrylate, and from about 1 to about 10% by weight methacrylic acid.

As described herein-above, in one embodiment of the invention, the core stage polymer contains co-polymer having as co-polymerized units from 5 to 100%, based on the weight of the core stage polymer, of at least one ethylenically unsaturated monomer containing acid functionality, and from 0 to 95% by weight, based on the weight of the core stage polymer, of at least one nonionic monoethylenically unsaturated monomer; and the shell stage polymer is formed by polymerizing from about 90% by weight to about 99.9% by weight, based on the total weight of shell stage polymer, of at least one nonionic monoethylenically unsaturated monomer, and from about 0.1% by weight to about 10% by weight, based on the total weight of shell stage polymer, of an acid-functional monoethylenically unsaturated monomer. In this embodiment, when the particle size of the core stage polymer is from about 130 nm to about 2.0 micrometer, the acid-functional monoethylenically unsaturated monomer is preferably added to the polymerization of the shell stage polymer over the 100% of the total shell stage monomer feed, based on the total weight of the shell stage monomer feed, more preferably over the first 50% of the feed, even more preferably over the first 25% of the feed, and most preferably over the first 10% of the feed. When the particle size of the core stage polymer is less than about 130 nm, the acid-functional monoethylenically unsaturated monomer is preferably added to the polymerization of the shell stage polymer over the 50% of the total shell stage monomer feed, based on the total weight of the shell stage monomer feed, more preferably over the first 25% of the feed, and most preferably over the first 10% of the feed.

The hollow sphere polymer system must either (1) contain a shell stage monomer system containing at least 1% by weight acid functional monomer, the balance of which may be a nonionic monoethylenically unsaturated co-monomer, such as those mentioned herein-above for the core stage polymer; or (2) involve the swelling of the hollow sphere polymer in the presence of a solvent. The preferred amount of acid functional monomer in the monomer system used to prepare the shell stage polymer is from 5 to 10% by weight when solvent is not used, and from about 1 to 2% by weight when solvent is used.

When solvent is used, it assists in penetration of the shell by the fixed or permanent base. Suitable amounts of solvent are from 1 to 100 parts by weight, based on 100 parts by weight hollow sphere polymer, preferably from 5-10 parts by weight. Suitable solvents are any which will plasticize the shell, for example, hexanol, ethanol, 3-hydroxy-2,2,4-trimethylpentyl isobutyrate, toluene, mixtures of solvents, and the like. The solvent can be added either before, after, or with the addition of the base. In certain cases the shell stage monomer system itself can function as the solvent for the shell stage polymer.

Within the scope of the invention are, among others, shell stage polymers which completely encapsulate the core stage polymer; shell stage polymers which substantially, but incompletely encapsulate the core stage polymer; polymers that are swollen to provide a particle with at least one pore communicating between the surface of the particle and the interior, i.e., core or void, of the particle; polymer particles having multiple cores; multistaged polymers wherein the core polymer is a precursor to the acid-functionality containing core polymer of this invention and is subsequently converted to the acid-functionality containing core polymer of this invention by means such as hydrolysis of the core polymer according to the teachings of US Patent Nos. 5,041,464; 5,157,084; and 5,216,044, whether before, during, or after shell polymer formation and the core polymer is contacted with a fixed or permanent base, during or after the hydrolysis.

In one embodiment of the invention, the shell stage polymer is crosslinked. The crosslinking level is preferably from at least 2 mol percent, more preferably from at least 5%, based on the total mole of monomer used in the hollow sphere polymer. Crosslinking in the shell can be derived from the use of one or more polyethylenically unsaturated monomers. Suitable polyethylenically unsaturated monomers include those described herein-above for the core stage polymer. Alternatively, crosslinking of the shell stage polymer may be derived from the use of one or more multi-functional monomers to provide post-polymerization crosslinking of the shell. The multi-functional monomers contain at least one functional group capable of vinyl-copolymerization, and at least one functional group capable of reaction with suitable reactive molecules. Suitable reactive molecules include, for example, amines, diamines, amino acids and aminoalkyltialkoxysilanes; optionally followed by the addition of other reactive molecules: aldehydes (such as formaldehyde) dialdehydes (such as glutaric dialdehyde), hydrazines and dihydrazines (such as succinic dihydrazine) to form post-polymerization crosslinked sol-gels.

Examples of suitable functional groups and reactive molecules for post-polymerization crosslinking of the shell stage polymer, as well as multi-functional monomers suitable for post-polymerization crosslinking, are illustrated, without limitation, in European Patent Application EP 1092421.

The multi-stage polymer particles containing the core and shell stage polymers are prepared by sequential emulsion polymerization methods, which are well known in the art, for example as described in United States Patent No. 4,594,363. By "sequential emulsion polymerization" is meant herein that the homo- or co-polymers of one stage of the polymer are prepared in aqueous medium, by an emulsion polymerization process, in the presence of the dispersed polymer particles of a polymer stage previously formed by emulsion polymerization, such that the previously formed emulsion polymers are increased in size by deposition thereon of emulsion polymerized product of one, or more, successive monomer charges that are introduced into the medium containing the dispersed particles of the preformed emulsion polymer. Each stage of the hollow sphere polymer may be made in a single stage, or step, of the sequential polymerization, or may be made by a plurality of steps in sequence.

In the sequential emulsion polymerization with which the present invention is concerned, the term "seed" polymer is used to refer to an aqueous emulsion polymer dispersion, which may be the dispersion containing the first-formed polymer stage, or it may be the emulsion polymer dispersion obtained at the end of any subsequent stage, except the final stage of the sequential polymerization. Thus, a core stage polymer which is intended to be encapsulated by one, or more, subsequent stages of emulsion polymerization, may itself be termed a seed polymer for the next stage. Likewise, a seed polymer may be utilized to form the nuclei on which the core stage polymer is formed.

A water-soluble free radical initiator may be utilized in the aqueous emulsion polymerization. Suitable water-soluble free radical initiators include hydrogen peroxide; tert-butyl peroxide; alkali metal persulfates such as sodium, potassium and lithium persulfate; ammonium persulfate; and mixtures of such initiators with a reducing agent. Reducing agents include: sulfites, such as alkali metal metabisulfite, hydrosulfite, and hyposulfite; sodium formaldehyde sulfoxylate; and reducing sugars such as ascorbic acid and isoascorbic acid. The amount of initiator is preferably from 0.01 to 3 % by weight, based on the total amount of monomer and in a redox system the amount of reducing agent is preferably from 0.01 to 3 % by weight based on the total amount of monomer. The temperature may be in the range of about 10°C to 100°C. In the case of the persulfate systems, the temperature is preferably in the range of 60°C to 90°C. In the redox system, the temperature is preferably in the range of 30°C to 70°C. The type and amount of initiator may be the same or different in the various stages of the multi-stage polymerization.

One or more nonionic or anionic emulsifiers, or surfactants, may be used, either alone or together. Examples of suitable nonionic emulsifiers include tert-octylphenoxyethylpoly(39)-ethoxyethanol, dodecyloxypoly(10)ethoxyethanol, nonylphenoxyethyl-poly(40)ethoxyethanol, polyethylene glycol 2000 monooleate, ethoxylated castor oil, fluorinated alkyl esters and alkoxylates, polyoxyethylene (20) sorbitan monolaurate, sucrose monococoate, di(2-butyl)phenoxypoly(20) ethoxyethanol, hydroxyethylcellulosepolybutyl acrylate graft copolymer, poly(ethylene oxide)poly(butyl acrylate) block copolymer, block copolymers of propylene oxide and ethylene oxide, 2,4,7,9-tetramethyl-5-decyne-4,7-diol ethoxylated with 30 moles of ethylene oxide, N-polyoxyethylene(20)lauramide, N-lauryl-N-polyoxyethylene(3)amine and poly(10)ethylene glycol dodecyl thioether. Examples of suitable anionic emulsifiers include sodium lauryl sulfate, sodium dodecylbenzenesulfonate, potassium stearate, sodium dioctyl sulfosuccinate, sodium dodecyldiphenyloxide disulfonate, nonylphenoxyethylpoly(1)ethoxyethyl sulfate ammonium salt, sodium styrene sulfonate, sodium dodecyl allyl sulfosuccinate, linseed oil fatty acid, sodium or ammonium salts of phosphate esters of ethoxylated nonylphenol, sodium octoxynol-3-sulfonate, sodium cocoyl sarcocinate, sodium 1-alkoxy-2-hydroxypropyl sulfonate, sodium alpha-olefin (C₁₄C₁₆)sulfonate, sulfates of hydroxyalkanols, tetrasodium N-(1,2-dicarboxy ethyl)-N-octadecylsulfo-succinamate, disodium N-octadecylsulfosuccinamate, disodium alkylamido polyethoxy sulfosuccinate, disodium ethoxylated nonylphenol half ester of sulfosuccinic acid and the sodium salt of tert-octylphenoxyethoxypoly(39) ethoxyethyl sulfate. The one or more surfactants are generally used at a level of from 0 to 3 % based on the weight of the multi-stage polymer. The one or more surfactants can be added prior to the addition of any monomer charge, during the addition of a monomer charge or a combination thereof. In certain monomer/emulsifier systems for forming the shell, the tendency to produce gum or coagulum in the reaction medium may be reduced or prevented by the addition of about 0.05% to about 2.0% by weight, based on total weight of the shell polymer, of emulsifier without detriment to the deposition of the polymer formed on the previously formed core particles.

The amount of emulsifier may be zero, in the situation wherein a persulfate initiator is used, to 3 % by weight, based on the weight of total weight of the core polymer. By carrying out the emulsion polymerization while maintaining low levels of emulsifier, the subsequent stages of polymer-formation deposit the most-recently formed polymer on the existing dispersed polymer particles resulting from the preceding step or stage. As a general rule, the amount of emulsifier should be kept below that corresponding to the critical micelle concentration for a particular monomer system, but while this limitation is preferable and produces a unimodal product, it has been found that in some systems the critical micelle concentration of the emulsifier may be exceeded somewhat without the formation of an objectionable or excessive number of dispersed micelles or particles. It is for the purpose of controlling the number of micelles during the various stages of polymerization so that the deposition of the subsequently formed polymer in each stage occurs upon the dispersed micelles or particles formed in the previous stages, that the concentration of emulsifier is kept low.

The viscosity- average molecular weight of the polymer formed in a given stage may range from 100,000, or lower if a chain transfer agent is used, to several million molecular weight. When 0.1 % by weight to 20% by weight, based on the weight of the monomer, of a polyethylenically unsaturated monomer mentioned herein-above is used in making the core, the molecular weight is increased whether or not crosslinking occurs. The use of the polyethylenically unsaturated monomer reduces the tendency of the core polymer to dissolve when the multistaged polymer is treated with a swellant for the core. If it is desired to produce a core having a molecular weight in the lower part of the range, such as from 500,000 down to as low as about 20,000, it is frequently most practical to do so by avoiding the polyethylenically unsaturated monomers and using a chain transfer agent instead, such as 0.05% to 2% or more thereof, examples being alkyl mercaptans, such as sec-butyl mercaptan.

The amount of polymer deposited to form shell polymer is generally such as to provide an overall size of the multistage polymer particle of from 70 nm to 4.5 micrometer, preferably from 100 nm to 3.5 micrometer, more preferably from 200 nm to 2.0 micrometer, in unswollen condition, whether the shell polymer is formed in a single stage, or in a plurality of stages. In order to minimize the dry density of the final product, it is preferable to deposit only as much shell polymer as is needed to fully encapsulate the core.

The multi-stage polymer containing the core and shell stage polymers is swollen when the particles are subjected to a fixed or permanent base capable of swelling the core, resulting in the formation of the hollow sphere polymer. The swelling, or expansion, of the core may involve partial merging of the outer periphery of the core into the pores of the inner periphery of the shell and also partial enlargement or bulging of the shell and the entire particle overall. Suitable swelling agents are those which, in the presence of the multistage emulsion polymer, are capable of permeating the shell and swelling the core. By "fixed or permanent base" is meant herein a nonvolatile hard base, such as a metal hydroxide such as, for example, sodium hydroxide, potassium hydroxide, lithium hydroxide, strontium hydroxide, barium hydroxide. Preferred are sodium hydroxide and potassium hydroxide. The fixed or permanent base differs from volatile bases, such as ammonia, ammonium hydroxide, amines, salts of weak acids, which to some greater or lesser degree evaporate from the emulsion, either at ambient temperatures, or upon drying, and which have a pKb<7 (in water at 25 °C). Solvents, such as, for example, ethanol, hexanol, octanol, Texanol® solvent and those described in U.S. Patent 4,594,363, may be added to aid in fixed or permanent base penetration.

For the reasons noted herein-above, hollow sphere polymers are not currently utilized during the manufacture of decorative laminates. Despite the subjection of the hollow sphere polymer to the wet-end conditions of, among other things, high temperature and/or humidity, or the subjection of the formed paper to the even harsher conditions of decorative laminate processing, the fixed base-swollen hollow sphere polymer, when used in conjunction with a pigment is still able to impart to a decorative laminate product the improvements typically associated with fixed base-swollen hollow sphere polymers, often at a lower cost than is achievable where costly pigments, such as titanium dioxide, are utilized without a hollow sphere polymer.

In the preferred embodiment of the invention, a composition containing the hollow sphere polymer is incorporated into a decorative laminate paper during the wet-end formation of the decorative laminate paper. By "wet-end" is meant herein, the part of the decorative laminate paper processing, during which a predominantly cellulosic fiber pulp slurry is formed into a wet sheet on a paper machine, by techniques that are well known in the art. The hollow sphere polymer and at least one pigment, along with other ingredients, as necessary, are added to, and mixed with the slurry, which is then formed into a wet sheet of paper that contains, or incorporates, the hollow sphere polymer. Any suitable pigment may be used, however titanium dioxide is preferred. The decorative laminate paper is dried, and then impregnated with a crosslinking resin. Suitable resins include, for example, thermosetting resins containing phenoplasts and aminoplasts, such as, for example urea formaldehyde and melamine formaldehyde, and the like. By "impregnation" is meant that the paper is at least partially, preferably completely saturated with the crosslinking resin. Pressure, and heat, are applied to the crosslinking resin-impregnated decorative laminate paper, causing the resin to cure and harden, forming the decorative laminate. Typical temperatures applied to the crosslinking resin-impregnated decorative laminate paper are in the range of from 100°C to 300°C, preferably from 125°C to 250°C, more preferably from 140°C to 200°C. The resulting decorative laminate has improved opacity, above that obtainable in a decorative laminate prepared utilizing only a pigment, as well as lower cost, where a costly pigment, such as titanium dioxide, is used.

In a different embodiment of the invention, the decorative laminate paper is formed, and coated with a composition containing the hollow sphere polymer and at least one pigment, before or after drying the paper. The decorative laminate paper is then impregnated with a crosslinking resin of the type mentioned in the preferred embodiment herein-above. Pressure, and heat, are applied to the crosslinking resin-impregnated decorative laminate paper, causing the resin to cure, and harden, forming the decorative laminate. Typical temperatures applied to the crosslinking resin-impregnated decorative laminate paper are as mentioned in the embodiment directly herein-above.

The following examples illustrate specific aspects and particular embodiments of the invention which, however, in not to be construed as limited thereby.

A sodium-hydroxide swollen hollow sphere polymer (HSP), and a refined wood pulp and pigment slurry, are mixed to provide a blend containing a ratio of 20/60/20 hollow sphere pigment to wood pulp to TiO2 based on dry weight. This blend is diluted to a 0.2% solids dispersion under agitation and a paper sample is formed on the CTP (Centre Technique de Papier) Retention Former.

The paper sample thus formed is dried in an oven at 95°C at 50% relative humidity for 10 minutes. This drying process is repeated at a range of temperatures (50 to 90°C), relative humidities (20 to 80%), and drying times (2 to 20 minutes).

The resulting paper is impregnated with a crosslinking resin, and then heated under pressure, and dried to form a decorative laminate. The decorative laminate containing the hollow sphere polymer has a higher opacity than the decorative laminate that contains no hollow sphere polymer.

| **Example:** | **Comparative Eg.1** | **Comparative Eg.2** | **Eg.3** | **Eg.4** |
|---|---|---|---|---|
| Slurry pigment and HSP content | 100% TiO2 | 67% TiO2/ 33%CaCO3 | 33% TiO2/ 45%HSP/ 22%CaCO3 | 45% TiO2/ 33%HSP/ 22%CaCO3 |
| Opacity | 91.5 | 90.5 | 93.3 | 92.9 |

## Claims

1. A method of preparing a decorative laminate, comprising the steps of:
(I) preparing a paper by:
(a) providing a hollow sphere polymer made by:
i. forming a core stage polymer by polymerizing at least one ethylenically unsaturated monomer containing acid functionality,
ii. encapsulating said core stage polymer with a shell stage polymer, by emulsion polymerizing at least one ethylenically unsaturated monomer in the presence of said core stage polymer,
wherein said shell stage polymer permits penetration of a fixed or permanent base,
iii. contacting the resulting multi-stage polymer particles with fixed or permanent base,
wherein either (1) said shell stage polymer comprises at least 1% acid functional monomer, or (2) said contacting takes place in the presence of solvent;
(b) contacting said paper with a composition comprising said hollow sphere polymer, and at least one pigment; and
(c) drying said paper;
(II) impregnating said paper with a crosslinking resin;
(III) applying pressure to said paper; and
(IV) exposing said paper to temperatures of from 100°C to 300°C, to form the decorative laminate.

2. The method, according to claim 1, wherein said core stage polymer is formed by polymerizing from about 5% by weight to about 100% by weight, based on the total weight of core stage polymer, of said ethylenically unsaturated monomer containing acid functionality, and from 0% by weight to about 95% by weight, based on the total weight of core stage polymer, of at least one nonionic monoethylenically unsaturated monomer;
wherein said shell stage polymer is formed by polymerizing from about 90% by weight to about 99.9% by weight, based on the total weight of shell stage polymer, of at least one nonionic monoethylenically unsaturated monomer, and from about 0.1% by weight to about 10% by weight, based on the total weight of shell stage polymer, of an acid functional monoethylenically unsaturated monomer; and
wherein said acid-functional monoethylenically unsaturated monomer is added to the polymerization of said shell stage polymer over the 100% of the total shell stage monomer feed, when the particle size of said core stage polymer is from about 130 nm to about 2.0 micrometer.

3. The method, according to claim 1, wherein said core stage polymer is formed by polymerizing from about 5% by weight to about 100% by weight, based on the total weight of core stage polymer, of said ethylenically unsaturated monomer containing acid functionality, and from 0% by weight to about 95% by weight, based on the total weight of said core stage polymer, of at least one nonionic monoethylenically unsaturated monomer;
wherein said shell stage polymer is formed by polymerizing from about 90% by weight to about 99.9% by weight, based on the total weight of shell stage polymer, of at least one nonionic monoethylenically unsaturated monomer, and from about 0.1% by weight to about 10% by weight, based on the total weight of shell stage polymer, of an acid-functional monoethylenically unsaturated monomer; and
wherein said acid-functional monoethylenically unsaturated monomer is added to the polymerization of said shell stage polymer over the first 50% of the total shell stage monomer feed, when the particle size of said core stage polymer is less than about 130 nm.

4. The method of claim 1, wherein said shell stage polymer is crosslinked.

5. The method of claim 1, wherein said contacting of said paper comprises, incorporating said composition in said paper during the wet-end formation of said paper.

6. The method of claim 1, wherein said contacting of said paper comprises coating said paper with said composition.

7. A decorative laminate formed by the method of any one of claims 1-6.

## Patentansprüche

1. Verfahren zur Herstellung eines Dekorlaminats, umfassend die Schritte:
(I) des Herstellens eines Papiers mittels:
(a) des Bereitstellens eines Hohlkugelpolymers, hergestellt durch:
i. das Bilden eines Kernphase-Polymers durch das Polymerisieren mindestens eines ethylenisch ungesättigten Monomers, das Säurefunktionalität enthält,
ii. das Verkapseln des Kernphase-Polymers mit einem Hüllphase-Polymer durch das Emulsionspolymerisieren mindestens eines ethylenisch ungesättigten Monomers in der Gegenwart des Kernphase-Polymers,
wobei das Hüllphase-Polymer das Eindringen einer fixierten oder permanenten Base zuläßt,
iii. das Inkontaktbringen der resultierenden Mehrphase-Polymerteilchen mit der fixierten oder permanenten Base, wobei entweder (1) das Hüllphase-Polymer mindestens 1% säurefunktionelles Monomer umfasst oder (2) das Inkontaktbringen in der Gegenwart eines Lösungsmittels erfolgt;
(b) des Inkontaktbringens des Papiers mit einer Zusammensetzung, die das Hohlkugelpolymer und mindestens ein Pigment umfasst; und
(c) des Trocknens des Papiers;
(II) des Imprägnierens des Papiers mit einem Vernetzungsharz;
(III) des Anwendens von Druck auf das Papier und
(IV) des Aussetzens des Papiers Temperaturen von 100°C bis 300°C, um das Dekorlaminat zu bilden.

2. Verfahren nach Anspruch 1, wobei das Kernphase-Polymer durch das Polymerisieren von etwa 5 Gew.-% bis etwa 100 Gew.-%, basierend auf dem Gesamtgewicht des Kernphase-Polymers, des ethylenisch ungesättigten Monomers, das Säurefunktionalität enthält, und von 0 Gew.-% bis etwa 95 Gew.-%, basierend auf dem Gesamtgewicht des Kernphase-Polymers, mindestens eines nichtionischen monoethylenisch ungesättigten Monomers gebildet ist,
wobei das Hüllphase-Polymer durch das Polymerisieren von etwa 90 Gew.- % bis etwa 99.9 Gew.-%, basierend auf dem Gesamtgewicht des Hüllphase-Polymers, mindestens eines nichtionischen monoethylenisch ungesättigten Monomers und von etwa 0,1 Gew.-% bis etwa 10 Gew.-%, basierend auf dem Gesamtgewicht des Hüllphase-Polymers, eines säurefunktionellen monoethylenisch ungesättigten Monomers gebildet ist, und
wobei das säurefunktionelle monoethylenisch ungesättigte Monomer der Polymerisation des Hüllphase-Polymers über die 100% der gesamten Hüllphase-Monomer-Zufuhr zugegeben wird, wenn die Teilchengröße des Kernphase-Polymers von etwa 130 nm bis etwa 2,0 Mikrometer beträgt.

3. Verfahren nach Anspruch 1, wobei das Kernphase-Polymer durch das Polymerisieren von etwa 5 Gew.-% bis etwa 100 Gew.-%, basierend auf dem Gesamtgewicht des Kernphase-Polymers, des ethylenisch ungesättigten Monomers, das Säurefunktionalität enthält, und von 0 Gew.-% bis etwa 95 Gew.-%, basierend auf dem Gesamtgewicht des Kernphase-Polymers, mindestens eines nichtionischen monoethylenisch ungesättigten Monomers gebildet ist,
wobei das Hüllphase-Polymer durch das Polymerisieren von etwa 90 Gew.- % bis etwa 99.9 Gew.-%, basierend auf dem Gesamtgewicht des Hüllphase-Polymers, mindestens eines nichtionischen monoethylenisch ungesättigten Monomers und von etwa 0,1 Gew.-% bis etwa 10 Gew.-%, basierend auf dem Gesamtgewicht des Hüllphase-Polymers, eines säurefunktionellen monoethylenisch ungesättigten Monomers gebildet ist, und
wobei das säurefunktionelle monoethylenisch ungesättigte Monomer der Polymerisation des Hüllphase-Polymers über die ersten 50% der gesamten Hüllphase-Monomer-Zufuhr zugegeben wird, wenn die Teilchengröße des Kernphase-Polymers weniger als etwa 130 nm beträgt.

4. Verfahren nach Anspruch 1, wobei das Hüllphase-Polymer vernetzt ist.

5. Verfahren nach Anspruch 1, wobei das Inkontaktbringen des Papiers das Inkorporieren der Zusammensetzung in dem Papier während der Nasspartie-Bildung des Papiers umfasst.

6. Verfahren nach Anspruch 1, wobei das Inkontaktbringen des Papiers das Beschichten des Papiers mit der Zusammensetzung umfasst.

7. Dekorlaminat, gebildet durch das Verfahren nach einem der Ansprüche 1 bis 6.

## Revendications

1. Procédé de préparation d'un stratifié décoratif comprenant les étapes de :
(I) préparation d'un papier par :
(a) fourniture d'un polymère à sphères creuses produit par :
i. formation d'un polymère de stade de noyau par polymérisation d'au moins un monomère éthyléniquement insaturé contenant une fonctionnalité acide,
ii. encapsulation dudit polymère de stade de noyau avec un polymère de stade d'enveloppe, par polymérisation en émulsion d'au moins un monomère éthyléniquement insaturé en présence dudit polymère de stade de noyau,
où ledit polymère de stade d'enveloppe permet la pénétration d'une base fixée ou permanente,
iii. mise en contact des particules de polymère multi-stade résultantes avec une base fixée ou permanente,
où (1) ledit polymère de stade d'enveloppe comprend au moins 1 % de monomère à fonctionnalité acide, ou (2) ladite mise en contact a lieu en présence de solvant ;
(b) mise en contact dudit papier avec une composition comprenant ledit polymère à sphères creuses, et au moins un pigment ; et
(c) séchage dudit papier ;
(II) imprégnation dudit papier avec une résine réticulante ;
(III) application d'une pression audit papier ; et
(IV) exposition dudit papier à des températures de 100°C à 300°C pour former le stratifié décoratif.

2. Procédé selon la revendication 1, où ledit polymère de stade de noyau est formé par polymérisation d'environ 5 % en poids à environ 100 % en poids, sur la base du poids total du polymère de stade de noyau, dudit monomère éthyléniquement insaturé contenant une fonctionnalité acide, et de 0 % en poids à environ 95 % en poids, sur la base du poids total du polymère de stade de noyau, d'au moins un monomère monoéthyléniquement insaturé non ionique ;
où ledit polymère de stade d'enveloppe est formé par polymérisation d'environ 90 % en poids à environ 99,9 % en poids, sur la base du poids total du polymère de stade d'enveloppe, d'au moins un monomère monoéthyléniquement insaturé non ionique, et d'environ 0,1 % en poids à environ 10 % en poids, sur la base du poids total du polymère de stade d'enveloppe, d'un monomère monoéthyléniquement insaturé à fonctionnalité acide ; et
où ledit monomère monoéthyléniquement insaturé à fonctionnalité acide est ajouté à la polymérisation dudit polymère de stade d'enveloppe sur les 100 % de l'alimentation en monomères de stade d'enveloppe totale, quand la taille de particule dudit polymère de stade de noyau est d'environ 130 nm à environ 2,0 µm.

3. Procédé selon la revendication 1, où ledit polymère de stade de noyau est formé par polymérisation d'environ 5 % en poids à environ 100 % en poids, sur la base du poids total du polymère de stade de noyau, dudit monomère éthyléniquement insaturé contenant une fonctionnalité acide, et de 0 % en poids à environ 95 % en poids, sur la base du poids total dudit polymère de stade de noyau, d'au moins un monomère monoéthyléniquement insaturé non ionique ;
où ledit polymère de stade d'enveloppe est formé par polymérisation d'environ 90 % en poids à environ 99,9 % en poids, sur la base du poids total du polymère de stade d'enveloppe, d'au moins un monomère monoéthyléniquement insaturé non ionique, et d'environ 0,1 % en poids à environ 10 % en poids, sur la base du poids total du polymère de stade d'enveloppe, d'un monomère monoéthyléniquement insaturé à fonctionnalité acide ; et
où ledit monomère monoéthyléniquement insaturé à fonctionnalité acide est ajouté à la polymérisation dudit polymère de stade d'enveloppe sur les 50 premiers % de l'alimentation en monomères de stade d'enveloppe totale, quand la taille de particule dudit polymère de stade de noyau est inférieure à environ 130 nm.

4. Procédé selon la revendication 1, où ledit polymère de stade d'enveloppe est réticulé.

5. Procédé selon la revendication 1, où ladite mise en contact dudit papier comprend l'incorporation de ladite composition dans ledit papier pendant la formation dudit papier à l'extrémité humide.

6. Procédé selon la revendication 1, où ladite mise en contact dudit papier comprend le revêtement dudit papier avec ladite composition.

7. Stratifié décoratif formé par le procédé selon l'une quelconque des revendications 1-6.
